

## UNITED STATES PATENT OFFICE

JOSEPH R. C. MARSH, OF CHICAGO, ILLINOIS

## IRON OR STEEL AND PROCESS OF MAKING OR TREATING SAME

No Drawing.

Application filed January 10, 1920. Serial No. 350,550.

My invention relates to the manufacture of alloy steel, or to the treatment thereof during the manufacturing process or later operations thereon.

5 An object of my invention is to provide a treatment for iron or steel in the ladle, or crucible or other suitable retainer which will impart thereto certain qualities which have not heretofore been obtained. Thus it is my object to not only increase the toughness and tenacity of the iron or steel, to add to its tensile, torsional and transverse strength and at the same time to increase its strength in alternating stress and resistance to abrasion 10 while keeping the compressive strength high as well as the elastic limits high in all its strengths, but to give it a fine grain and great homogeneity.

Other objects and advantages will appear 15 herein.

In carrying my invention into effect I make use of copper, chromium and nickel, with which the iron or steel is treated while in a molten state, with results as hereinafter 20 described. The carbon, silicon, manganese, sulphur, phosphorus and other elements may be varied to meet certain requirements as in the case of other steels. The metallic copper raises the elastic limit and ultimate load in 25 both steel and iron, gives resiliency and to some extent hardness, and the chromium also adds to the ultimate load and gives the quality of resistance to shock or impact. The chromium and the copper both refine the grain. 30 This alloy can be readily rolled, forged or otherwise mechanically formed.

35 Deoxidization is by the addition of titanium, vanadium, or boron, usually in the form of a ferro alloy. The silicon, manganese, carbon, phosphorus and sulphur contents are acquired according to the customary methods.

40 The copper can be added to the cold or molten charge or to the molten metal, after the furnace begins to operate, sufficient time being allowed in the latter case to allow the copper to melt and properly mix with the molten metal. The chromium should be added preferably in the form of ferro-chromium after 45 the manganese, or about fifteen minutes be-

fore pouring. The proportion of ferro-chromium will depend upon its chromium content so as to provide the chromium proportion of the formula in any instance. The nickel is added to the cold or molten charge 50 or to the molten metal after the furnace begins to operate and before the manganese is added.

As an example of the percentages of the ingredients which give good results, I may cite the following:

|                   | Per cent |
|-------------------|----------|
| Chromium about    | .85      |
| Copper about      | .85      |
| Nickel about      | 1.70     |
| Silicon about     | .15      |
| Manganese about   | .25      |
| Sulphur about     | .03      |
| Phosphorous about | .03      |
| Carbon about      | .35      |
| Iron about        | 95.79    |

70 This table gives the proportion of the weight of each ingredient as compared with the total weight of the complete resultant product. It will be understood that it is the treatment 75 by adding the chromium, copper and nickel, and the peculiar steps attending this treatment which distinguish my invention from heretofore known processes of making or treating steel; and that a substance made up 80 of any or all of the ingredients of the above list excepting the copper, chromium and nickel, or a substance including any other ingredient with iron such as to give it the ordinary properties of any of the well-known 85 variations of commercial alloy steel is to be considered as a ferro metal or steel. Thus, my formula, according to the above example, may be briefly stated as

|                   | Per cent |
|-------------------|----------|
| Chromium about    | .85      |
| Copper about      | .85      |
| Nickel about      | 1.70     |
| Ferro metal about | 96.60    |

90 The properties due to the nickel in this alloy are: the better alloying of the copper and the chromium, the reduction of segregation of copper and chromium, and the reduction in size of the different crystals in the 95 alloy.

An alloy manufactured substantially according to the information above set forth is not merely useful in a cast form, but is readily rolled into any of the usual shapes given to 5 iron or steel; whereas any marked variation from the proportions of the elements, especially the copper, chromium and nickel, as herein given, precludes the mechanical working of this alloy, as by rolling or forging, 10 due to hot shortness, especially if the proportion of the copper is raised. This has been determined by me in actual practice.

To obtain an appreciable effect in accordance with my invention, the copper and 15 chromium should not be used in proportions much less than about .30% each. On the other hand, if much more than about 1.50% copper is used, the steel is made so "hot short" that it cannot be successfully rolled; and if 20 more than 3.00% of chromium be used the steel will cost more than the increased results obtained from such excess of chromium would justify. In any instance, the proportion of nickel should not be materially less 25 than the aggregate of the proportions of copper and chromium. Nickel will mix physically with both copper and chromium, and when used in the proportion of two parts by weight of nickel to one part by weight each 30 of copper and chromium, the best results are obtained. However, with maximums of 1.50% of copper and 3.00% chromium, as high as 6.00% nickel may be used.

The product is highly satisfactory in use 35 where much more expensive steels have heretofore been found indispensable, as for instance, as tool steel, rails, car axles, tension members of railway cars and bridges.

The superiority of my alloy steel over open 40 hearth steel has been demonstrated by The Bethlehem Steel Company at Bethlehem, Pennsylvania, as shown by the following comparison taken from tests made by its metallurgical department in its report of 45 September 17, 1919:

| Open hearth steel                |                            | Marsh                                       |
|----------------------------------|----------------------------|---------------------------------------------|
| Yield point in tension           | 35,000 lbs. to square inch | 95,000 lbs. to square inch                  |
| Cost per ton                     | \$56                       | \$74                                        |
| 1" round rod 100 ft. long weighs | 267 lbs.                   | 5/8" round rod 100 ft. long weighs 104 lbs. |
| Cost of rod                      | \$7,476                    | \$3,848                                     |
| Yield point in tension of 1" rod | 27,489 lbs.                | Yield point in tension 5/8" rod 29,146 lbs. |

50 55 Saving in cost \$3,628. Saving in weight of 163 lbs. and a gain in strength of 1,657 lbs. stress.

The correctness of the above test was confirmed by the Lewis Institute, of Chicago, Illinois, and by the Bureau of Standards, 60 Washington, D. C.

65 It will be understood that while I have mentioned some uses for which my improved product is most satisfactory and have specified certain ingredients and proportions of ingredients, including those of the copper,

chromium and nickel, in order to make a full and clear disclosure of my invention, nevertheless there is the possibility of some departure from the precise ingredients and proportions as well as many fields of usefulness not specifically mentioned herein without departing from the scope or spirit of my invention, which, having thus fully set forth, I define in the following claims:

70

1. An alloy steel containing the following 75 elements: copper from .30% to 1.50%, chromium from .30% to 3.00%, nickel from .60% to 6.00% and ferro metal or steel from 98.80% to 90.50% and having non-hot-short rollable properties when combined from the minimum to the maximum range, substantially as described.

80

2. An alloy containing, in proportion to the total weight of the alloy, a ferro metal about 96.60%, copper and chromium each 85 about .85% and nickel about 1.70%.

85

3. An alloy containing in proportion to the total weight of the alloy, chromium about .85%, copper about .85%, nickel about 1.70%, silicon about .15%, manganese about .25%, sulphur about .03%, phosphorus about .03%, carbon about .35%, and iron about 95.79%.

90

4. The process of treating a ferro metal which consists in mixing in a melted state said metal and copper and nickel, and afterward mixing chromium with the combination of said metal and copper and nickel while said combination and the chromium are in a melted state.

95

5. The process of treating a ferro metal 100 which consists in mixing in a melted state said metal and copper and nickel, then mixing with the combination of said metal and copper and nickel a proper proportion of manganese while said combination and said manganese are in a melted state, and then mixing with this combination chromium while this combination and said chromium are in a melted state.

105

JOSEPH R. C. MARSH. 110

115

120

125

130